

3,281,369

## CORROSION INHIBITING COMPOSITIONS

Robert Walter Wynn, Easton, Pa., assignor to General Aniline & Film Corporation, New York, N.Y., a corporation of Delaware  
No Drawing. Filed June 26, 1963, Ser. No. 290,612  
9 Claims. (Cl. 252—146)

The present invention relates, in general, to argano phosphates and, in particular, to tripropargyl phosphate which finds immediate and practical utility as a corrosion inhibitor in lubricating oils, hydraulic fluids, antifreeze, dry cleaning compositions and acid-metal cleaning or pickling solutions.

When operations such as metal cleaning, scale removal and the like are carried out on an industrial scale, acid solutions are employed to accomplish the purpose. Acids which find utility in this respect include inorganic and organic acids, such as hydrochloric, sulfuric, phosphoric, hydrofluoric, citric, oxalic, sulfamic acids, and the like.

In almost all of the aforesaid operations, it is usually necessary to incorporate a corrosion inhibitor into the acid solution to prevent or decrease the attack of the acid upon the base metal. In order for a corrosion inhibitor to be considered an effective candidate for incorporation into an acid cleaning solution it should, in addition to inhibiting or preventing corrosion of the base metal, function to decrease or inhibit hydrogen embrittlement of the base metal; be stable with respect to color and precipitation in acid solutions. However, according to some heretofore customary practices, certain commercial inhibitors which are derivatives of propargyl, alcohol as well as propargyl alcohol itself, when incorporated into acid cleaning solutions, have a decided tendency to turn back and form insoluble polymeric precipitates in the solutions. In addition, corrosion inhibition tests of propargyl alcohol and certain propargyl alcohol derivatives indicate that the use of such compounds does not inhibit the change in crystallinity and hence embrittlement of the metal to the desired degree.

Accordingly, it is an object of this invention to provide a corrosion inhibiting composition which does not substantially change color upon use.

Another object of the invention resides in the provision of corrosion inhibiting compositions which have a substantially high degree of stability with regard to precipitation upon standing.

Yet another object of this invention is directed to the feature of a corrosion inhibiting composition which is capable of substantially preventing or lessening the phenomenon known as hydrogen embrittlement.

Still other objects of the invention will become more readily apparent from the following detailed description of the invention.

The above objects of the invention are readily accomplished by incorporating into acid-cleaning compositions a corrosion inhibiting amount of tripropargyl phosphate.

Extensive testing of tripropargyl phosphate as an agent in an acid solution for preventing or decreasing the attack on a base metal while being subjected to metal-cleaning or scale removal operations, have indicated a lower weight loss occurs as a result of acid corrosion with tripropargyl phosphate as compared with other commercially acceptable corrosion inhibitors. A further advantage of tripropargyl phosphate as a component in a corrosion inhibiting composition resides in its apparent effectiveness in preventing or lessening hydrogen embrittlement.

The results of the testing indicated above of tripropargyl phosphate as compared with other commercially acceptable corrosion inhibitors is reflected in the subsequent

Table I with various acid solutions based on 2.5 weight percent of additive based on 100 percent of acid employed. In comparing the properties and advantages of tripropargyl phosphate as an additive component in acid-cleaning solutions with other commercially acceptable inhibitors with respect to stability and inhibiting of corrosion and hydrogen embrittlement, the following tests were performed:

## Hydrogen embrittlement inhibition

The method employed, essentially that of C. A. Zapffe et al., described in Metals Technology, January (1946), pp. 281-312 (discontinued 1948, now issued as Journal of Metals), treats stainless steel wire AISI 440 C., 0.060" in diameter in the pickling acid for 15 minutes at 77° C. then bends the wire around a  $\frac{1}{16}$ " pin until breakage occurs. The angle of breakage or bend tolerance is an indication of hydrogen embrittlement inhibition, the higher values indicating greater inhibition activity.

## Corrosion inhibition

The test method employed to measure the effectiveness of test compounds as corrosion inhibitors is based on the weight loss which occurs after a test panel is immersed in a test acid solution for a given period of time. In the tests conducted, the results of which are reported below, 1" x 2" panels of mild steel (1010 type) are immersed in 10 percent hydrochloric and sulfuric acids test solutions containing 0.25 weight percent (2.5 weight percent based on 100 percent acid) of the test corrosion inhibitors for two hours at 77° C. The panels are then removed from the solutions, flushed, dried and measured by weight loss.

## Stability

The stability of tripropargyl phosphate and other additives with regard to color and precipitation in concentrated hydrochloric acid was carried out by adding from 0.5 to 1.0 weight percent of the additives to the acid solution with or without mixing. The test solutions were examined visibly over a period of time and changes in color and composition recorded.

The following Table I reflects the data obtained in tests of various corrosion inhibitors including tripropargyl phosphate. The table also reflects the values obtained with tests of solutions which did not contain any corrosion inhibitor.

TABLE I

| Test Inhibitor                                                                                                | Hydrogen Embrittlement, Break Angle |         | Corrosion Mild Steel, Percent Wt. Loss |         |
|---------------------------------------------------------------------------------------------------------------|-------------------------------------|---------|----------------------------------------|---------|
|                                                                                                               | 10% H <sub>2</sub> SO <sub>4</sub>  | 10% HCl | 10% H <sub>2</sub> SO <sub>4</sub>     | 10% HCl |
| None                                                                                                          | 45                                  | 63      | 4.3                                    | 11.4    |
| Propargyl Alcohol                                                                                             | 64                                  | 109     | 2.0                                    | 0.09    |
| Propargyl Alcohol plus 1.98 moles of Ethylene Oxide, (CH=CH <sub>2</sub> OCH <sub>2</sub> ) <sub>2</sub> CHOH | 51                                  | 103     | 1.9                                    | 0.4     |
| Glycidyl Ether of Polymerized Propargyl Alcohol                                                               | 68                                  | 93      | 5.6                                    | 0.3     |
| Tripropargyl Phosphate, CH=CH <sub>2</sub> OCH <sub>2</sub> CH <sub>2</sub> OH                                | 50                                  | 97      | 3.1                                    | 0.6     |
| C <sub>2</sub> H <sub>5</sub>                                                                                 | 73                                  | 108     | 0.5                                    | 0.1     |
| CH=CH <sub>2</sub> OCH <sub>2</sub> CHOH                                                                      | 74                                  | 109     | 1.7                                    | 0.3     |
| CH=CH <sub>2</sub> NHCH <sub>2</sub> CH <sub>2</sub> OH                                                       | 63                                  | 103     | 2.0                                    | 0.3     |
| Antarate 3482 <sup>1</sup>                                                                                    | 47                                  | 94      | 13.2                                   | 0.8     |
| Blank Untreated                                                                                               | 41                                  | 42      | 0.05                                   | 0.4     |
|                                                                                                               | 101                                 | 101     |                                        |         |

<sup>1</sup> A mixture of aromatic amines with propargyl alcohol.

The following Table II illustrates the results obtained in stability tests of various propargyl alcohol derivatives as stabilizing additives for analytical grade 37 percent hydrochloric acid.

TABLE II.—STABILIZATION OF ANALYTICAL GRADE 37% HCl WITH PROPARGYL  
ALCOHOL DERIVATIVES  
[Time, days]

| Ex. No. | Chemicals Added                                                                              | 0                        | 1              | 2              |
|---------|----------------------------------------------------------------------------------------------|--------------------------|----------------|----------------|
| 1.....  | 0.5% Tripropargyl <sup>1</sup> Phosphate.....                                                | Clear and colorless..... | No change..... | No change..... |
| 2.....  | Repeat of 1 <sup>2</sup> .....                                                               | do.....                  | do.....        | Do.....        |
| 3.....  | 0.5% Glycidyl Ether of Polymerized Propargyl Alcohol.....                                    | Darkens slightly.....    | do.....        | Do.....        |
| 4.....  | 0.5% Dipropargyloxymethyl Methanol.....                                                      | do.....                  | do.....        | Do.....        |
| 5.....  | 1% $\text{CH} \equiv \text{CCH}_2\text{SCH}_2\text{CH}_2\text{OH}$ .....                     | do.....                  | do.....        | do.....        |
| 6.....  | 1% $\text{CH} \equiv \text{CCH}_2\text{OCH}_2\text{CH}(\text{C}_2\text{H}_5)\text{OH}$ ..... | do.....                  | do.....        | do.....        |
| 7.....  | 1% $\text{CH} \equiv \text{CCH}_2\text{OCH}_2\text{CH}(\text{CH}_3)\text{OH}$ .....          | do.....                  | do.....        | do.....        |
| 8.....  | 1% Antarctic 3481.....                                                                       | Very dark.....           | No change..... | No change..... |

  

| Ex. No. | 3              | 4                         | 5                 | 6              | 7               | 8                             |
|---------|----------------|---------------------------|-------------------|----------------|-----------------|-------------------------------|
| 1.....  | No change..... | No change.....            | No change.....    | No change..... | No change.....  | No change.....                |
| 2.....  | do.....        | do.....                   | do.....           | do.....        | do.....         | do.....                       |
| 3.....  | do.....        | Slightly cloudy.....      | do.....           | do.....        | Slight ppt..... | Slight ppt., yellow soln..... |
| 4.....  | do.....        | do.....                   | do.....           | do.....        | do.....         | Do.....                       |
| 5.....  | Darker.....    | Cloudy and very dark..... | Ppt. forming..... | do.....        | No change.....  | Much Ppt., very dark.....     |
| 6.....  | do.....        | Ppt. forming.....         | No change.....    | do.....        | do.....         | Ppt. in dark soln.....        |
| 7.....  | do.....        | do.....                   | do.....           | do.....        | do.....         | Do.....                       |
| 8.....  | No change..... | No change.....            | do.....           | do.....        | do.....         | Very dark but no ppt.....     |

<sup>1</sup> Still clear and colorless after 23 days.

<sup>2</sup> Still clear and colorless after 16 days.

The amount of tripropargyl phosphate to be employed to be effective in minimizing corrosion and hydrogen embrittlement and to provide stable acid solutions is not necessarily a critical feature of the invention. In general, effective corrosion inhibiting amounts range from 0.5 to 5 weight percent based on 100 percent acid and is, therefore, preferred.

The following example illustrates the preparation of the additive of the invention.

*Example 1.—Preparation of tripropargyl phosphate*

There was charged 168.0 grams (3 moles) propargyl alcohol, 404.8 grams (4 moles) triethyl amine, and 500 cc's. dry ether. At  $-5^\circ$  to  $-10^\circ$  C. there was added dropwise a solution of 153.0 grams (1 mole) phosphorus oxychloride in 100 cc's. dry ether in 1.5 hours. The mixture was stirred one hour longer at  $-10$  to  $0^\circ$  C. The amine hydrochloride was removed by filtration and the ether removed under aspiration vacuum. The residue was then heated to  $50^\circ$  C. under 0.2 mm. Hg pressure.

This residue was then heated to  $70^\circ$  C., with stirring, with 150 ml. distilled water. To this was added 150 cc's. benzene and the phases separated. The aqueous phase was extracted with two 100 cc. portions of benzene. The organic layers were combined and dried overnight at room temperature over Drierite. The desiccant was removed by gravity filtration and the benzene removed under aspirator vacuum. The residue was heated to  $60^\circ$  C. under 0.2 mm. Hg pressure. There remained 52.6 grams of a straw-yellow oil having a boiling point of  $111$ – $113^\circ$  C. at 0.08 mm. of Hg pressure and a refractive index ( $n_D^{25}$ ) of 1.4680–1.4684.

*Analysis.*— $\text{C}_9\text{H}_8\text{O}_4\text{P}$ :

|                                    | Cal'd.  | Found        |
|------------------------------------|---------|--------------|
| Percent C.....                     | 51.0    | 52.38        |
| Percent H.....                     | 4.25    | 5.42         |
| Percent P.....                     | 14.6    | 13.41; 13.48 |
| Acetylenic Hydrogen (mole/g.)..... | 0.01415 | 0.01408      |

The product obtained as described in the foregoing example was satisfactory for use without further purification and was employed as a corrosion inhibitor with the results given in Tables I and II above. It has been found that when tripropargyl phosphate was prepared at a substantially higher temperature than employed in the foregoing example, an impure highly colored (dark red) product was obtained. Such impure products are less

satisfactory as corrosion inhibitors, but can readily be purified and a good grade of corrosion inhibitor obtained by distillation under reduced pressures in the presence of a small amount of a free radical inhibitor, i.e., p-tert-butyl catechol.

Various other modifications and variations will be obvious to a person skilled in the art and it is to be understood that such modifications and variations are to be included in the purview of the application and the spirit and scope of the appended claims.

What is claimed is:

1. A metal cleaning composition consisting essentially of an acid selected from the group consisting of hydrochloric, sulfuric, phosphoric, hydrofluoric, citric, oxalic and sulfamic acids in an amount sufficient to clean metal, and 0.5 to 5 weight percent, based on 100 percent acid, of tripropargyl phosphate.
2. The composition of claim 1 wherein the acid is sulfamic acid.
3. The composition of claim 1 wherein the acid is oxalic acid.
4. The composition of claim 1 wherein the acid is citric acid.
5. The composition of claim 1 wherein the acid is hydrofluoric acid.
6. The composition of claim 1 wherein the acid is phosphoric acid.
7. The composition of claim 1 wherein the acid is sulfuric acid.
8. The composition of claim 1 wherein the acid is hydrochloric acid.
9. As a corrosion inhibitor, tripropargyl phosphate.

References Cited by the Examiner

UNITED STATES PATENTS

|           |         |                |                |
|-----------|---------|----------------|----------------|
| 2,080,299 | 5/1937  | Benning et al. | 260—461.312 XR |
| 2,224,695 | 12/1940 | Prutton        | 260—461.312 XR |
| 2,589,326 | 3/1952  | Oberright      | 260—461.312 XR |
| 3,049,496 | 8/1962  | Monroe et al.  | 252—146        |

OTHER REFERENCES

Foster et al., "Acetylenic Corrosion Inhibitors," Industrial and Engineering Chemistry, vol. 51, July 1959, pp. 825–828.

LEON D. ROSDOL, Primary Examiner.

JULIUS GREENWALD, Examiner.

W. E. SCHULZ, Assistant Examiner.